

## UNITED STATES PATENT OFFICE

2,448,169

## ZINC-TITANIUM-CADMIUM ALLOYS

Edward J. Boyle and Edmund A. Anderson, Palmerston, Pa., assignors to The New Jersey Zinc Company, New York, N. Y., a corporation of New Jersey

No Drawing. Application May 17, 1944,  
Serial No. 536,017

7 Claims. (Cl. 75—178)

1

This invention relates to zinc base alloys and more particularly to zinc base alloys containing titanium, and aims to provide an improved zinc base alloy containing titanium and cadmium.

The zinc base alloys of the invention contain from 0.01 to 1.6%, and preferably from 0.05 to 0.5%, titanium and are characterized by additionally containing from 0.05 to 1.5%, and preferably from 0.1 to 1%, cadmium. The balance of the alloy is zinc. Alloys of the invention may advantageously contain about 0.1% titanium, 0.3 to 0.6% cadmium, and the balance zinc. The zinc base of the alloys is preferably high grade zinc. Alloys of superior creep resistance, that is resistance to prolonged static loads well below the ultimate limit, and of fine grain size when cast result from the use, as the zinc base, of metal of high purity, such as zinc at least 99.99% pure. On the other hand, satisfactory alloys are obtained with zinc of the grade commonly used in the production of commercial rolled zinc, for example zinc metal containing 0.10% lead, 0.012% iron and 0.005% cadmium. The presence of 0.1% lead is sufficient, however, to impart to the alloys (as cast) a coarse, columnar grain structure similar to that of ordinary cast zinc. If the alloy is rolled or otherwise mechanically worked, the coarse grain structure of the cast alloy disappears, and the micro-structure and properties of the rolled or worked alloy are substantially independent of the grade or purity of the zinc metal of the types hereinbefore mentioned.

The alloys of the invention are particularly adapted for rolling. When transformed to sheet or strip by suitable rolling procedure, the alloys possess high creep resistance. The alloys may be hot rolled at metal temperatures of from 150 to 300° C., temperatures of from 200 to 240° C. giving very satisfactory results. The hot rolling may be a finishing operation consisting of say three or more passes through the rolls, and may be applied to metal either hot or cold rolled prior to the hot finishing. Cold rolling tends to decrease the creep resistance, but the characteristic high creep resistance can be substantially restored by subsequent heat treatment such, for example, as annealing for a short period at a temperature of from 150 to 400° C., annealing in oil for about five minutes at a temperature of about 275° C. giving very satisfactory results. Cold rolling, at least in the final stages, imparts to the alloy certain advantages, especially with respect to hardness. Alloys of the invention are to be considered cold rolled when the rolling (or other mechanical working) is carried out under thermal conditions resulting in a temperature of the rolled strip or sheet after the final rolling pass (final coil temperature) due simply to the mechanical working, and are to be considered hot rolled when the rolling is carried out under thermal condi-

tions resulting in a final coil temperature of from 150 to 300° C., and preferably from 200 to 240° C.

In the production of the alloys of the invention, it is preferable to prepare an intermediate zinc base alloy containing a relatively high proportion of titanium. Conveniently, the intermediate alloy may contain about 4% of titanium, and is prepared by heating a mixture of 96 parts of zinc and 4 parts of titanium in a clay-carborundum crucible at a temperature of 800° C. for about 8 hours. The intermediate alloy is cast into a thin slab and crushed to a convenient size for alloying. The final titanium content of the cast intermediate alloy usually does not depart far from the contemplated 4%. The contemplated titanium content of the alloy of the invention is then readily obtained by adding the calculated amount of the intermediate alloy to a predetermined weight of molten zinc. Cadmium, in amount calculated to give the desired content in the final alloy, may be added as such to the molten mixture of zinc and the intermediate zinc-titanium alloy, or the cadmium may be included in the zinc, or melted down with the zinc and intermediate zinc-titanium alloy.

The alloys of the invention are characterized by high creep resistance, dynamic ductility, tensile strength, tensile elongation and good bending properties. These characteristics of the alloys (among others) are shown in the following table. In the table, "H" is sclerometer hardness; "D. D." is dynamic ductility and is measured as the maximum depth in inches of a cup that can be formed by a standard plunger in an uncut sheet of the metal without fracture; "Tem." is percent temper, and is determined by the degree to which a standard test strip returns to its original position after being wrapped around a mandrel; "T. S." is tensile strength (with the grain) in pounds per square inch; "T. E." is tensile elongation (with the grain), in percent in a 2 inch test strip; and "C. R." is the creep rate or creep resistance (with the grain) expressed as the inverse creep rate (the more creep resistant alloy having the higher inverse creep rate) which is the number of units of time (days) required to produce an elongation or creep (with the grain) of one percent (i. e. days per percent) in a standard test piece when subjected to dead loads of 8,000 and 12,000 pounds (respectively) per square inch at constant room temperature (25° C.). The cold bend values represent the diameter of uncracked 180° bends in multiples of sheet thickness (gauge), and the lower values indicate better bending properties. "Cut and draw" is the result of an actual drawing operation carried out on a disc cut from the sheet, and the figures given represent the per cent decrease in diameter of the cup, as compared with the blank (per cent take-in). The columns headed by the single

asterisk (\*) and by the double asterisk (\*\*) are results obtained with test pieces as rolled, and as annealed for five minutes at 275° C. in oil, respectively. The titanium (Ti) and cadmium (Cd) contents of the alloys given in the table are the amounts of these alloying metals added to the zinc base which was high purity metal. The alloys were compounded in the manner hereinbefore described.

0.05 to 0.5% titanium, from 0.1 to 1% cadmium, and the balance zinc with not more than 0.1% lead as an impurity.

7. A zinc base alloy according to claim 6 containing about 0.1% titanium and from 0.3 to 0.6% cadmium.

EDWARD J. BOYLE.  
EDMUND A. ANDERSON.

Table

| Ti                                                                                                                                                                                               | Cd | Test Gauge | H                | D. D.              | Tem.           | Cold Bends |              | T. S.  | T. E.  | Creep Resistance   |                     | Cut and draw      |      |
|--------------------------------------------------------------------------------------------------------------------------------------------------------------------------------------------------|----|------------|------------------|--------------------|----------------|------------|--------------|--------|--------|--------------------|---------------------|-------------------|------|
|                                                                                                                                                                                                  |    |            |                  |                    |                | With Grain | Across Grain |        |        | 8,000 p. s. i.     | 12,000 p. s. i.     |                   |      |
| .1                                                                                                                                                                                               | .5 | .016       | (*) (**) 20 17.5 | (*) (**) .265 .300 | (*) (**) 55 48 | 3½ 3½      | (*) (**) 2 2 | 24,800 | 27,200 | (*) (**) 45.3 32.2 | (*) (**) 2.22 188.7 | (*) (**) .095 .66 | 43.9 |
| Rolling Treatment:<br>Slab heated to 230°-260° C., rough rolled to 0.09" in ten passes; cold rolled on warm rolls to 0.018" in five passes, final coil temperature 90-130° C.                    |    |            |                  |                    |                |            |              |        |        |                    |                     |                   |      |
| .1                                                                                                                                                                                               | .5 | .021       | 19 18            | .325 .320          | 45 44          | 2 3        | 2 2          | 26,900 | 28,900 | 40.0 34.5          | 7.04 303.0          | .17 .81           | 44.9 |
| Rolling Treatment:<br>Slab heated to 230-260°C., rough rolled to 0.09" in ten passes; cold coil rolled on hot rolls to 0.018" in three passes, final coil temperature 160-185° C.                |    |            |                  |                    |                |            |              |        |        |                    |                     |                   |      |
| .1                                                                                                                                                                                               | .5 | .0175      | 23 18            | .255 .310          | 55 47          | 5 2½       | 2 2          | 24,600 | 27,700 | 43.6 41.0          | 1.87 256.4          | .042 1.03         |      |
| Rolling Treatment:<br>Slab heated to 220-240° C., rough rolled to 0.125" in ten passes; coil cold rolled on warm rolls to 0.036" in three passes; finally cold rolled to 0.018" in three passes. |    |            |                  |                    |                |            |              |        |        |                    |                     |                   |      |

\* As rolled. \*\* As annealed.

We claim:

1. A zinc base alloy characterized by high creep resistance and containing from 0.05 to 0.5% titanium, from 0.1 to 1% cadmium, and the balance zinc with not more than 0.1% lead as an impurity.

2. A zinc base alloy characterized by high creep resistance and containing about 0.1% titanium, from 0.3 to 0.6% cadmium, and the balance zinc with not more than 0.1% lead as an impurity.

3. A zinc base alloy characterized by high creep resistance and containing about 0.1% titanium, about 0.5% cadmium, and the balance zinc with not more than 0.1% lead as an impurity.

4. A cold rolled and annealed zinc base alloy characterized by high creep resistance and containing from 0.05 to 0.5% titanium, from 0.1 to 1% cadmium, and the balance zinc with not more than 0.1% lead as an impurity.

5. A zinc base alloy according to claim 4 containing about 0.1% titanium and from 0.3 to 0.6% cadmium.

6. A hot rolled zinc base alloy characterized by high creep resistance and containing from

## REFERENCES CITED

35 The following references are of record in the file of this patent:

## UNITED STATES PATENTS

| 40 | Number    | Name         | Date          |
|----|-----------|--------------|---------------|
|    | 1,020,512 | Rossi -----  | Mar. 19, 1912 |
|    | 1,888,567 | Pierce ----- | Nov. 22, 1932 |
|    | 2,048,288 | Pierce ----- | July 21, 1936 |
|    | 2,317,179 | Daesen ----- | Apr. 20, 1943 |

## FOREIGN PATENTS

| Number  | Country             | Date          |
|---------|---------------------|---------------|
| 125,397 | Great Britain ----- | Aug. 7, 1919  |
| 826,013 | France -----        | Dec. 27, 1937 |

## 50 OTHER REFERENCES

55 Circular of the Bureau of Standards, No. 395, "Zinc and Its Alloys," 1931, page 27, published by U. S. Gov't. Printing Office, Washington, D. C.

Metals Handbook, 1939 edition, pages 1737, 1765, published by American Society for Metals, Cleveland, Ohio.

**Certificate of Correction**

Patent No. 2,448,169.

August 31, 1948.

**EDWARD J. BOYLE ET AL.**

It is hereby certified that errors appear in the printed specification of the above numbered patent requiring correction as follows:

Columns 3 and 4, in the table, description of the rolling treatment immediately below the first horizontal row of figures, for the words "cold rolled" read *cold coil rolled*; in the second horizontal row of figures, last column, under the heading "Cut and draw", insert the figures 46.9; in the third horizontal row of figures, under the heading "T. E.", for "43.6" read 43.7; in the last horizontal description of rolling treatment, for "coil cold rolled" read *cold coil rolled*;

and that the said Letters Patent should be read with these corrections therein that the same may conform to the record of the case in the Patent Office.

Signed and sealed this 14th day of December, A. D. 1948.

[~~SEAL~~]

**THOMAS F. MURPHY,**  
*Assistant Commissioner of Patents.*